# EUROPEAN PATENT APPLICATION

(11) **EP 2 278 406 A1**
(43) Date of publication of application: **26.01.2011**
(21) Application number: 10169608.6
(22) Date of filing: 15.07.2010
(51) Int. Cl.: G03G 5/147

(54) **Photoreceptor outer layer**

(30) Priority: 20.07.2009 US 506194
(71) Applicant: Xerox Corporation, Rochester, New York 14644 (US)
(72) Inventor: Kim, Woo Soo, Oakville Ontario L6H 0C7 (CA); Hu, Nan-Xing, Oakville Ontario L6H 6B4 (CA); Gagnon, Yvan, Mississauga Ontario L5L1K2 (CA); Junginger, Johann, Toronto Ontario M6S 3T9 (CA)
(74) Representative: De Anna, Pier Luigi

(57) **Abstract**

The presently disclosed embodiments relate generally to layers that are useful in imaging apparatus members and components, for use in electrophotographic, including digital, apparatuses. Embodiments pertain to an improved electrophotographic imaging member incorporating an outer layer having a nano- to micron-scale pattern imprinted into its surface to lower friction with the cleaning blade and improve print quality and performance.

## Description

### BACKGROUND

The presently disclosed invention relates generally to layers that are useful in imaging apparatus members and components, for use in electrophotographic, including digital, apparatuses. More particularly, the embodiments pertain to an improved electrophotographic imaging member comprising an outer layer having a nano- to micron-scale pattern imprinted into its surface to lower friction with the cleaning blade and improve print quality and performance. The embodiments also pertain to methods for making the improved electrophotographic imaging member.

In electrophotographic printing, the charge retentive surface, typically known as a photoreceptor, is electrostatically charged, and then exposed to a light pattern of an original image to selectively discharge the surface in accordance therewith. The resulting pattern of charged and discharged areas on the photoreceptor form an electrostatic charge pattern, known as a latent image, conforming to the original image. The latent image is developed by contacting it with a finely divided electrostatically attractable powder known as toner. Toner is held on the image areas by the electrostatic charge on the photoreceptor surface. Thus, a toner image is produced in conformity with a light image of the original being reproduced or printed. The toner image may then be transferred to a substrate or support member (e.g., paper) directly or through the use of an intermediate transfer member, and the image affixed thereto to form a permanent record of the image to be reproduced or printed. Subsequent to development, excess toner left on the charge retentive surface is cleaned from the surface. The process is useful for light lens copying from an original or printing electronically generated or stored originals such as with a raster output scanner (ROS), where a charged surface may be imagewise discharged in a variety of ways.

The described electrophotographic copying process is well known and is commonly used for light lens copying of an original document. Analogous processes also exist in other electrophotographic printing applications such as, for example, digital laser printing or ionographic printing and reproduction where charge is deposited on a charge retentive surface in response to electronically generated or stored images.

To charge the surface of a photoreceptor, a scorotron charging device or a contact type charging device has been used. The contact type charging device includes a conductive member which is supplied a voltage from a power source with a D.C. voltage superimposed with a A.C. voltage of no less than twice the level of the D.C. voltage. The charging device contacts the image bearing member (photoreceptor) surface, which is a member to be charged. The outer surface of the image bearing member is charged with the rubbing friction at the contact area. The contact type charging device charges the image bearing member to a predetermined potential. Typically the contact type charger is in the form of a roll charger such as that disclosed in U.S. Pat. No. 4,387,980.

Multilayered photoreceptors or imaging members have at least two layers, and may include a substrate, a conductive layer, an optional undercoat layer (sometimes referred to as a "charge blocking layer" or "hole blocking layer"), an optional adhesive layer, a photogenerating layer (sometimes referred to as a "charge generation layer," "charge generating layer," or "charge generator layer"), a charge transport layer, and an optional overcoating layer in either a flexible belt form or a rigid drum configuration. In the multilayer configuration, the active layers of the photoreceptor are the charge generation layer (CGL) and the charge transport layer (CTL). Enhancement of charge transport across these layers provides better photoreceptor performance. Multilayered flexible photoreceptor members may include an anti-curl layer on the backside of the substrate, opposite to the side of the electrically active layers, to render the desired photoreceptor flatness.

Print defects due to cleaning failure are one of the main issues in xerographic sub-systems. Such defects are typically observed when a low wear overcoated photoreceptor is used. For example, the defects often occur at a very early stage and is caused by blade damage and non-uniform wear of photoreceptor due to high friction and poor interactions between the cleaning blade and the photoreceptor. In another example, a print artifact known as paper edge ghost (PEG) is associated with differential positive charge stress from the transfer station in xerography. The visible ghost artifact correlates with a measurable difference in photo-induced discharge curve (PIDC). Thus, there is a need for an improved imaging layer that achieves extended service lifetime and does not suffer from the above-described problems.

The term "photoreceptor" or "photoconductor" is generally used interchangeably with the terms "imaging member." The term "electrophotographic" includes "electrostatographic" and "xerographic." The terms "charge transport molecule" are generally used interchangeably with the terms "hole transport molecule."

### SUMMARY

In one embodiment, there is provided an imaging member comprising a substrate, a photosensitive layer disposed on the substrate, and an outer layer disposed on the photosensitive layer, wherein the outer layer of the imaging member has a patterned surface comprising an array of periodically ordered indentations or protrusions on the surface of the outer layer.

In another embodiment, there is provided an imaging member comprising a substrate, a charge generation layer disposed on the substrate, and a charge transport layer disposed on the charge generation layer, wherein the charge transport layer has a patterned surface comprising an array of periodically ordered indentations or protrusions on the surface of the outer layer and further wherein the charge transport layer comprises a tertiary arylamine and an optional polymer binder present in a ratio amount of from about 10/90 to about 90/10.

In yet another embodiment, there is provided an image forming apparatus comprising an imaging member comprising a substrate, a photosensitive layer disposed on the substrate, and an outer layer disposed on the photosensitive layer, wherein the outer layer of the imaging member has a patterned surface comprising an array of periodically ordered indentations or protrusions on the surface of the outer layer, a charging unit that applies electrostatic charge on the imaging member, a developing unit that develops toner image onto the imaging member, a transfer unit that transfers the toner image from the imaging member to a media, and a cleaning unit that cleans the imaging member.

### BRIEF DESCRIPTION OF THE DRAWINGS

For a better understanding, reference may be made to the accompanying figures.

FIG. 1 is a cross-sectional view of an imaging member in a drum configuration according to the present embodiments;

FIG. 2 is a cross-sectional view of an imaging member in a belt configuration according to the present embodiments;

FIG. 3 is a diagram illustrating the steps for making an imaging member according to the present embodiments;

FIG. 4 is a graph illustrating torque reduction in imaging members made according to the present embodiments; and

FIG. 5 is a graph illustrating paper edge ghost (PEG) reduction in imaging members made according to the present embodiments.

### DETAILED DESCRIPTION

In the following description, reference is made to the accompanying drawings, which form a part hereof and which illustrate several embodiments. It is understood that other embodiments may be used and structural and operational changes may be made without departure from the scope of the present disclosure.

The presently disclosed embodiments are directed generally to an improved electrophotographic imaging member comprising an outer layer having a nano- to micron-scale pattern imprinted into its surface to lower friction with the cleaning blade and improve print quality and performance. The embodiments also pertain to methods for making the improved electrophotographic imaging member.

The exemplary embodiments of this disclosure are described below with reference to the drawings. The specific terms are used in the following description for clarity, selected for illustration in the drawings and not to define or limit the scope of the disclosure. The same reference numerals are used to identify the same structure in different figures unless specified otherwise. The structures in the figures are not drawn according to their relative proportions and the drawings should not be interpreted as limiting the disclosure in size, relative size, or location. In addition, Though the discussion will address negatively charged systems, the imaging members of the present disclosure may also be used in positively charged systems.

FIG. 1 is an exemplary embodiment of a multilayered electrophotographic imaging member having a drum configuration. As can be seen, the exemplary imaging member includes a rigid support substrate 10, an electrically conductive ground plane 12, an undercoat layer 14, a charge generation layer 18 and a charge transport layer 20. The rigid substrate may be comprised of a material selected from the group consisting of a metal, metal alloy, aluminum, zirconium, niobium, tantalum, vanadium, hafnium, titanium, nickel, stainless steel, chromium, tungsten, molybdenum, and mixtures thereof. The charge generation layer 18 and the charge transport layer 20 forms an imaging layer described here as two separate layers. In an alternative to what is shown in the figure, the charge generation layer may also be disposed on top of the charge transport layer. It will be appreciated that the functional components of these layers may alternatively be combined into a single layer.

FIG. 2 shows an imaging member having a belt configuration according to the embodiments. As shown, the belt configuration is provided with an anti-curl back coating 1, a supporting substrate 10, an electrically conductive ground plane 12, an undercoat layer 14, an adhesive layer 16, a charge generation layer 18, and a charge transport layer 20. An optional overcoat layer 32 and ground strip 19 may also be included. An exemplary photoreceptor having a belt configuration is disclosed in U.S. Patent No. 5,069,993.

Print defects due to cleaning failure and high torque are some of the main issues in xerographic sub-systems, and typically observed when a low wear overcoated photoreceptor is used. Positive charge stress from the transfer stations is associated with paper edge ghosts (PEG). More generally, when different areas of the photoreceptor undergo different stresses, there will be a differential aging effect which is characterized by a change in the performance of the photoreceptor in those areas. Such performance change can be characterized by measuring the photo-induced discharge curve (PIDC) of the photoreceptor. It is desirable to have a photoreceptor design which is robust against differential aging, such as PEG, as the typical countermeasure to when PEG is encountered in the field is to replace the photoreceptor.

In the present embodiments, it is discovered that one manner in which to address these problems is to impart unique surface morphology on the photoreceptor. For example, using an overcoated photoreceptor with a rough surface created by mechanical polish provides a surface that helps smooth interaction between the cleaning blade and the photoreceptor, thus minimizing blade damage and non-uniform photoreceptor wear. As the printing continues, the photoreceptor will generate its natural rough surface, and consequently maintains good interaction with the cleaning blade even after the initial surface structure is worn away. As for belt photoreceptor application, it has also been demonstrated previously that a polished photoreceptor belt exhibited low ghosting level. However, creating the desired surface through mechanical polish requires a repetitive process that takes additional time, is costly, and lacks of control of the surface morphology.

The present embodiments provide a xerographic photoreceptor that includes a nano- to micron-scale surface-structured outer layer by employing a micro/nano imprinting method. In embodiments, the imprinted outer layer may be an overcoat or a charge transport layer. The imprinting provides a uniform roughened surface to the outer layer, that is, roughened such that the surface is marked by irregularities, protuberances, or ridges, and is not smooth. In addition, the roughness is homogenous in degree, or regular and even throughout the surface of the outer layer. This imprinted surface offers lower friction with the cleaning blade, and thus improved print quality and smoother interaction to minimize blade damage. The imprinted surface also reduces paper edge ghosting (charge stress cycling) of the xerographic photoreceptor. The surface offers lower differential aging when subjected to positive charge stress cycling. Thus, it is expected that the controlled photoreceptor morphology helps extend customer replacement units (CRU) life.

The micro/nano imprinting method can give homogenously periodic and wide patterns on the outer layer surface. Depending on the design of the flexible mold, the morphology of the surface may be controlled, resulting in a "designed roughened" surface for improved system interactions, for instance, reduced torque, minimized blade damage and minimized non-uniform photoreceptor wear. In this disclosure, it is also shown that photoreceptors which employ outer layers with the imprinted surface pattern on a nano- or micron-scale exhibit improved PEG behavior. The present embodiments provide a method for forming a photoreceptor outer layer that comprises providing a mold for imprinting, providing an outer layer coating for being imprinted, laying the mold over the outer layer coating for contacting until the mold and the outer layer coating is cross-linked, and subsequently removing the mold from the outer layer coating such that an outer layer comprising a surface pattern imprinted on a nano- or micron-scale is formed. In embodiments, the mold is fabricated by printing a pattern on a nano- or micron-scale on a substrate to produce a master pattern, and curing a flexible material onto the master pattern to form the mold.

In the disclosed method, the substrate used for the master pattern may comprise any suitable substrate such as, for example, polyethylene terephtalate, silicon, glass, MYLAR, plastics, mixtures thereof, and the like. In addition, the flexible material may comprise polysiloxane, polyurethane, polyester, fluorosilicone and mixtures thereof, and the like. In embodiments, the outer layer coating formed on the photoreceptor comprises, in embodiments, an organic film and a cross-linking agent, such as for example, an amino resin, sol-gel siloxane, melamine resin, and the like, and mixtures thereof.

In particular, the fabrication steps for the flexible mold and micro/nano imprinting, and the scanning electron microscope (SEM) images corresponding to the steps, are shown in FIG. 3. A mold is fabricated by inkjet printing a nano- or micron-scale pattern onto a substrate, such as polyethylene terephtalate, to create a photo-mask master pattern 5. A flexible material, such as polydimethylsiloxane (PDMS) materials, is then cured onto the master pattern to form the mold 10. After removal from the photo-mask master pattern 15, the flexible mold is used to lay over an outer layer coating-first semi cross-linking 20 and eventually fully cross-linking 25-after the flexible mold and outer layer coating are fully contacted. The mold is subsequently removed, resulting in an outer layer having an imprinted surface pattern on a nano- or micron-scale 30.

In one embodiment, there is provided a method for forming an imaging member having a patterned surface in the outer layer, comprising providing a mold for imprinting, wherein the mold comprises a pattern on one face of the mold, comprising a array of periodically ordered protrusions or indentations, providing an imaging member comprising a substrate and, disposed on the substrate, an soft outer layer coating for being imprinted, pressing the patterned face of the mold and the outer layer coating of the imaging member together in a manner that the pattern structure of the mold is replicated onto outer layer coating, and hardening the outer layer coating to form a patterned structure on the surface of the imaging member. The hardening step is realized by a process selected from the group consisting of thermal drying, thermal curing, photo-induced curing, electron beam cuing, and mixtures thereof.

In particular embodiments, the outer layer coating of the imaging member comprises a charge transport component and a polymer binder. In such embodiments, the charge transport component comprises a tertiary arylamine selected from the group consisting of N,N'-diphenyl-N,N'-bis(3-methylphenyl)-(1,1'-biphenyl)-4,4'-diamine, N,N'-diphenyl-N,N'-bis(4-methylphenyl)-(1,1'-biphenyl)-4,4'-diamine, N,N,N',N'-tetrakis(4-methylphenyl)- 1,1'-biphenyl)-4,4'-diamine, N,N'-bis(4-butylphenyl)-N,N'-di-p-tolyl-[p-terphenyl]-4,4'-diamine, and N,N'-bis(4-butylphenyl)-N,N'-di-m-tolyl-[p-terphenyl]-4,4'-diamine, and mixtures thereof.

Furthermore, the outer layer coating may, in embodiments, comprise a curable composition comprising charge transport component and a curing agent. The curing agent may be selected from the group consisting of a melamine-formaldehyde resin, a phenol resin, an isocyalate or a masking isocyalate compound, an acrylate resin, a polyol resin, or the mixture thereof.

In one embodiment, the outer layer is an overcoat layer that comprises a cross-linked composition further comprising a charge transport component. In embodiments, the cross-linked composition is the result of curing and polymerization of a charge transport component further comprising a tertiary arylamine having at least a curable functional group selected from the group consisting of a hydroxyl, a hydroxymethyl, an alkoxymethyl, a hydroxyalkyl having from 1 to about 15 carbons, an acrylate, and the mixture thereof.

In embodiments, the mold may comprise an elastic material such as those selected from the group consisting of polysiloxane, polyurethane, polyester, fluoro-silicone, and mixtures thereof. The mold may further comprise, in embodiments, a substrate to support the pattern layer, and the substrate is made of a material selected from the group consisting of a metal, a polymer, a glass, a ceramic, and wood. In embodiments, a further step of applying a release agent onto the mold prior to the imprinting may be included. The release agent may comprise a low surface energy material.

In specific embodiments, there is provided an imaging member such that, positioned in between the substrate and the outer layer coating, there is positioned a charge generation layer comprising a photosensitive pigment selected from the group consisting of metal free phthalocyanine, titanyl phthalocyanine, chlorogallium phthalocyanine, hydroxygallium phthalocyanine, and a mixture of alkylhydroxy gallium phthalocyanine and hydroxygallium phthalocyanine, and a perylene, and the mixture thereof. The wherein said substrate is in a cylinder, a drum, or a belt configuration.

In further embodiments, the surface pattern may include specific shapes and dimensions. For example, the surface pattern design may comprise circles, rods, squares, triangles, polygons, mixtures thereof and the like. The dimensions may of a few nanometers scale to thousand microns scale. In embodiments, the surface pattern may include an array of indentations having a depth of from about 5 nanometers to about 5 microns, or from about 10 nanometers to about 5 microns, or from about 50 nanometers to about 5 microns, or from about 100 nanometers to about 2 microns. In further embodiments, each of the indentations has a perimeter from about 5 nanometers to about 200 microns. The indentations may be in the shape of circles, rods, squares, triangles, polygons, mixtures thereof and the like. The array of indentations is regularly positioned over the surface of the outer layer. These surface patterns serve as an air reservoir or gap between the outer layer and the charging effluents during process of charge stress cycling, and thus help reduce PEG. In other embodiments, the surface pattern comprises one or more indentations, and may further comprise an array of indentations that are uniformly positioned across the surface of the outer layer. The indentations may include specific dimensions. For example, in one embodiment, the array of indentations having a diameter of from about 5 nanometers to about 100 microns, or from about 10 nanometers to about 100 microns. In other embodiments, the array of indentations have a center-to-center distance of from about 5 nanometers to about 500 microns, or from about 10 nanometers to about 100 microns. The surface pattern may include indentations being of equidistance from one another in an evenly distributed pattern across the surface of the outer layer of the photoreceptor and forming a uniform roughened pattern on the surface of the photoreceptor.

In addition, the surface pattern may comprise an array of protrusions or bumps. These bumps may likewise be in the shape of circles, rods, squares, triangles, polygons, mixtures thereof and the like. The dimensions would remain the same as discussed for the indentations above, however, the dimension for depth will be reversed to a dimension for height. Thus, the protrusions may have a height of from about 5 nanometers to about 5 microns, or from about 10 nanometers to about 5 microns, or from about 50 nanometers to about 5 microns, or from about 100 nanometers to about 2 microns. The methods for making the protrusions would likewise comprise the same steps as discussed for the indentations, but the shapes (*e.g*., concave versus convex) of the master pattern and mold would be reversed accordingly.

In further embodiments, there is provided an imaging forming apparatus comprising an imaging member as described above, a charging unit that applies electrostatic charge on the imaging member, a developing unit that develops toner image onto the imaging member, a transfer unit that transfers the toner image from the imaging member to a media, and a cleaning unit that cleans the imaging member. In such embodiments, the indentations or protrusions may have a depth or height of from about 0.1 micrometer to about 5 microns, and the array of indentations or protrusions may each have a perimeter of from about 0.1 micrometer to about 200 microns. In additional embodiments, the array of indentations or protrusions may further have a center-to-center distance of from about 0.5 micrometer to about 200 microns. In embodiments, the cleaning unit of the image forming apparatus may comprise a blade-type cleaner comprised of an elastic polymer.

The Overcoat Layer

Other layers of the imaging member may include, for example, an optional over coat layer 32. An optional overcoat layer 32, if desired, may be disposed over the charge transport layer 20 to provide imaging member surface protection as well as improve resistance to abrasion. In embodiments, the overcoat layer 32 may have a thickness ranging from about 0.1 micrometer to about 25 micrometers or from about 1 micrometer to about 15 micrometers, or in a specific embodiment, about 3 to about 10 micrometers. These overcoating layers may include a charge transport component and an optional organic polymers or inorganic polymers.

In embodiments, the overcoat layer may include a charge transport component. In particular embodiments, the overcoat layer comprises a charge transport component comprised of a tertiary arylamine containing a substituent capable of self cross-linking or reacting with the polymer resin to form cured composition. Specific examples of charge transport component suitable for overcoat layer comprise the tertiary arylamine with a general formula of wherein Ar¹, Ar², Ar³, and Ar⁴ each independently represents an aryl group having about 6 to about 30 carbon atoms, Ar⁵ represents aromatic hydrocarbon group having about 6 to about 30 carbon atoms, and k represents 0 or 1, and wherein at least one of Ar¹, Ar², Ar³ Ar⁴ , and Ar⁵ comprises a substituent selected from the group consisting of hydroxyl (-OH), a hydroxymethyl (-CH₂OH), an alkoxymethyl (-CH₂OR, wherein R is an alkyl having 1 to about 10 carbons), a hydroxylalkyl having 1 to about 10 carbons, and mixtures thereof. In other embodiments, Ar¹, Ar², Ar³, and Ar⁴ each independently represent a phenyl or a substituted phenyl group, and Ar⁵ represents a biphenyl or a terphenyl group.

Additional examples of charge transport component which comprise a tertiary arylamine include the following: and the like, wherein R is a substituent selected from the group consisting of hydrogen atom, and an alkyl having from 1 to about 6 carbons, and *m* and *n* each independently represents 0 or 1, wherein *m*+*n* > 1. In specific embodiments, the overcoat layer may include an additional curing agent to form a cured overcoat composition. Illustrative examples of the curing agent may be selected from the group consisting of a melamine-formaldehyde resin, a phenol resin, an isocyalate or a masking isocyalate compound, an acrylate resin, a polyol resin, or the mixture thereof.

In specific embodiments, the overcoat layer is imprinted on its surface with a nano- to micron-scale pattern. The imprinted surface offers numerous unexpected benefits such as, for example, lower friction with the cleaning blade, improved print quality and smoother interaction to minimize blade damage, and consequently longer service life.

The present embodiments thus provide an imaging member comprising a substrate, an imaging layer disposed on the substrate, and an overcoat layer disposed on the imaging layer, wherein the overcoat layer comprises a surface pattern imprinted on a nano- or micron-scale. The surface pattern may include specific shapes and dimensions. For example, the surface pattern may comprise circles, rods, squares, triangles, oval, polygons, mixtures thereof and the like. In one embodiment, the surface pattern may include one or more indentations. In embodiments, the surface pattern may include an array of indentations having a depth of from about 5 nanometers to about 5 microns, or from about 10 nanometers to about 5 microns, or from about 50 nanometers to about 5 microns, or from about 100 nanometers to about 2 microns. In embodiments, the surface pattern comprises an array of indentations having a diameter of from about 5 nanometers to about 100 microns, or from about 10 nanometers to about 100 microns. In other embodiments, the array of indentations has a center-to-center distance of from about 5 nanometers to about 500 microns, or from about 10 nanometers to about 100 microns. The surface pattern may include indentations being of equidistance from one another in an evenly distributed pattern across the surface of the overcoat layer of the photoreceptor and forming a uniform roughened pattern on the surface of the photoreceptor. The indentations may be in the shape of circles, rods, squares, triangles, polygons, mixtures thereof, and the like. Alternative patterns may include periodic or non-periodic hole arrays, two-dimensional crystalline hexagonal patterns, rectangular arrays of patterns or quasi-crystalline array of patterns.

The present embodiments are made by a method that comprises forming the overcoat layer having the imprinted surface pattern through use of a fabricated mold. For example, the present embodiments provide for a method for forming a photoreceptor overcoat layer, comprising providing a mold for imprinting, wherein the mold is fabricated by printing a pattern on a nano- or micron-scale on a substrate to produce a master pattern, and curing a flexible material onto the master pattern to form the mold, providing an overcoat layer coating for being imprinted, laying the mold over the overcoat layer coating for contacting until the mold and the overcoat layer coating is cross-linked, and removing the mold from the overcoat layer coating such that an overcoat layer comprising a surface pattern imprinted on a nano- or micron-scale is formed. It was discovered that an imaging member made from this method exhibited a reduction in torque. For example, an imaging member comprising the overcoat layer having the surface pattern exhibits from about 10% to about 90% reduction in torque as compared to an imaging member comprising an overcoat layer without the surface pattern. A specific embodiment exhibits about a 40% reduction in torque as compared to an imaging member comprising an overcoat layer without the surface pattern.

The Substrate

The photoreceptor support substrate 10 may be opaque or substantially transparent, and may comprise any suitable organic or inorganic material having the requisite mechanical properties. The entire substrate can comprise the same material as that in the electrically conductive surface, or the electrically conductive surface can be merely a coating on the substrate. Any suitable electrically conductive material can be employed, such as for example, metal or metal alloy. Electrically conductive materials include copper, brass, nickel, zinc, chromium, stainless steel, conductive plastics and rubbers, aluminum, semitransparent aluminum, steel, cadmium, silver, gold, zirconium, niobium, tantalum, vanadium, hafnium, titanium, nickel, niobium, stainless steel, chromium, tungsten, molybdenum, paper rendered conductive by the inclusion of a suitable material therein or through conditioning in a humid atmosphere to ensure the presence of sufficient water content to render the material conductive, indium, tin, metal oxides, including tin oxide and indium tin oxide, and the like. It could be single metallic compound or dual layers of different metals and/ or oxides.

The substrate 10 can also be formulated entirely of an electrically conductive material, or it can be an insulating material including inorganic or organic polymeric materials, such as MYLAR, a commercially available biaxially oriented polyethylene terephthalate from DuPont, or polyethylene naphthalate available as KALEDEX 2000, with a ground plane layer 12 comprising a conductive titanium or titanium/zirconium coating, otherwise a layer of an organic or inorganic material having a semiconductive surface layer, such as indium tin oxide, aluminum, titanium, and the like, or exclusively be made up of a conductive material such as, aluminum, chromium, nickel, brass, other metals and the like. The thickness of the support substrate depends on numerous factors, including mechanical performance and economic considerations.

The substrate 10 may have a number of many different configurations, such as for example, a plate, a cylinder, a drum, a scroll, an endless flexible belt, and the like. In the case of the substrate being in the form of a belt, as shown in FIG. 2, the belt can be seamed or seamless. In embodiments, the photoreceptor herein is in a drum configuration.

The thickness of the substrate 10 depends on numerous factors, including flexibility, mechanical performance, and economic considerations. The thickness of the support substrate 10 of the present embodiments may be at least about 500 micrometers, or no more than about 3,000 micrometers, or be at least about 750 micrometers, or no more than about 2500 micrometers.

The Ground Plane

The electrically conductive ground plane 12 may be an electrically conductive metal layer which may be formed, for example, on the substrate 10 by any suitable coating technique, such as a vacuum depositing technique. Metals include aluminum, zirconium, niobium, tantalum, vanadium, hafnium, titanium, nickel, stainless steel, chromium, tungsten, molybdenum, and other conductive substances, and mixtures thereof. The conductive layer may vary in thickness over substantially wide ranges depending on the optical transparency and flexibility desired for the electrophotoconductive member. Accordingly, for a flexible photoresponsive imaging device, the thickness of the conductive layer may be at least about 20 Angstroms, or no more than about 750 Angstroms, or at least about 50 Angstroms, or no more than about 200 Angstroms for an optimum combination of electrical conductivity, flexibility and light transmission.

Regardless of the technique employed to form the metal layer, a thin layer of metal oxide forms on the outer surface of most metals upon exposure to air. Thus, when other layers overlying the metal layer are characterized as "contiguous" layers, it is intended that these overlying contiguous layers may, in fact, contact a thin metal oxide layer that has formed on the outer surface of the oxidizable metal layer. Generally, for rear erase exposure, a conductive layer light transparency of at least about 15 percent is desirable. The conductive layer need not be limited to metals. Other examples of conductive layers may be combinations of materials such as conductive indium tin oxide as transparent layer for light having a wavelength between about 4000 Angstroms and about 9000 Angstroms or a conductive carbon black dispersed in a polymeric binder as an opaque conductive layer.

The Hole Blocking Laver

After deposition of the electrically conductive ground plane layer, the hole blocking layer 14 may be applied thereto. Electron blocking layers for positively charged photoreceptors allow holes from the imaging surface of the photoreceptor to migrate toward the conductive layer. For negatively charged photoreceptors, any suitable hole blocking layer capable of forming a barrier to prevent hole injection from the conductive layer to the opposite photoconductive layer may be utilized. The hole blocking layer may include polymers such as polyvinylbutryral, epoxy resins, polyesters, polysiloxanes, polyamides, polyurethanes and the like, or may be nitrogen containing siloxanes or nitrogen containing titanium compounds such as trimethoxysilyl propylene diamine, hydrolyzed trimethoxysilyl propyl ethylene diamine, N-beta-(aminoethyl) gamma-amino-propyl trimethoxy silane, isopropyl 4-aminobenzene sulfonyl, di(dodecylbenzene sulfonyl) titanate, isopropyl di(4-aminobenzoyl)isostearoyl titanate, isopropyl tri(N-ethylamino-ethylamino)titanate, isopropyl trianthranil titanate, isopropyl tri(N,N-dimethylethylamino)titanate, titanium-4-amino benzene sulfonate oxyacetate, titanium 4-aminobenzoate isostearate oxyacetate, [H₂N(CH₂)₄]CH₃Si(OCH₃)₂, (gamma-aminobutyl) methyl diethoxysilane, and [H₂N(CH₂)₃]CH₃Si(OCH₃)₂ (gamma-aminopropyl) methyl diethoxysilane, as disclosed in U.S. Pat. Nos. 4,338,387, 4,286,033 and 4,291,110.

General embodiments of the undercoat layer may comprise a metal oxide and a resin binder. The metal oxides that can be used with the embodiments herein include, but are not limited to, titanium oxide, zinc oxide, tin oxide, aluminum oxide, silicon oxide, zirconium oxide, indium oxide, molybdenum oxide, and mixtures thereof. Undercoat layer binder materials may include, for example, polyesters, MOR-ESTER 49,000 from Morton International Inc., VITEL PE-1 00, VITEL PE-200, VITEL PE-200D, and VITEL PE-222 from Goodyear Tire and Rubber Co., polyarylates such as ARDEL from AMOCO Production Products, polysulfone from AMOCO Production Products, polyurethanes, and the like.

The hole blocking layer should be continuous and have a thickness of less than about 0.5 micrometer because greater thicknesses may lead to undesirably high residual voltage. A hole blocking layer of between about 0.005 micrometer and about 0.3 micrometer is used because charge neutralization after the exposure step is facilitated and optimum electrical performance is achieved. A thickness of between about 0.03 micrometer and about 0.06 micrometer is used for hole blocking layers for optimum electrical behavior. The blocking layer may be applied by any suitable conventional technique such as spraying, dip coating, draw bar coating, gravure coating, silk screening, air knife coating, reverse roll coating, vacuum deposition, chemical treatment and the like. For convenience in obtaining thin layers, the blocking layer is applied in the form of a dilute solution, with the solvent being removed after deposition of the coating by conventional techniques such as by vacuum, heating and the like. Generally, a weight ratio of hole blocking layer material and solvent of between about 0.05:100 to about 0.5:100 is satisfactory for spray coating.

The Charge Generation Layer

The charge generation layer 18 may thereafter be applied to the undercoat layer 14. Any suitable charge generation binder including a charge generating/ photoconductive material, which may be in the form of particles and dispersed in a film forming binder, such as an inactive resin, may be utilized. Examples of charge generating materials include, for example, inorganic photoconductive materials such as amorphous selenium, trigonal selenium, and selenium alloys selected from the group consisting of selenium-tellurium, selenium-tellurium-arsenic, selenium arsenide and mixtures thereof, and organic photoconductive materials including various phthalocyanine pigments such as the X-form of metal free phthalocyanine, metal phthalocyanines such as vanadyl phthalocyanine and copper phthalocyanine, hydroxy gallium phthalocyanines, chlorogallium phthalocyanines, titanyl phthalocyanines, quinacridones, dibromo anthanthrone pigments, benzimidazole perylene, substituted 2,4-diamino-triazines, polynuclear aromatic quinones, enzimidazole perylene, and the like, and mixtures thereof, dispersed in a film forming polymeric binder. Selenium, selenium alloy, benzimidazole perylene, and the like and mixtures thereof may be formed as a continuous, homogeneous charge generation layer. Benzimidazole perylene compositions are well known and described, for example, in U.S. Patent No. 4,587,189. Multi-charge generation layer compositions may be used where a photoconductive layer enhances or reduces the properties of the charge generation layer. Other suitable charge generating materials known in the art may also be utilized, if desired. The charge generating materials selected should be sensitive to activating radiation having a wavelength between about 400 and about 900 nm during the imagewise radiation exposure step in an electrophotographic imaging process to form an electrostatic latent image. For example, hydroxygallium phthalocyanine absorbs light of a wavelength of from about 370 to about 950 nanometers, as disclosed, for example, in U.S. Pat. No. 5,756,245.

Any suitable inactive resin materials may be employed as a binder in the charge generation layer 18, including those described, for example, in U.S. Patent No. 3,121,006. Organic resinous binders include thermoplastic and thermosetting resins such as one or more of polycarbonates, polyesters, polyamides, polyurethanes, polystyrenes, polyarylethers, polyarylsulfones, polybutadienes, polysulfones, polyethersulfones, polyethylenes, polypropylenes, polyimides, polymethylpentenes, polyphenylene sulfides, polyvinyl butyral, polyvinyl acetate, polysiloxanes, polyacrylates, polyvinyl acetals, polyamides, polyimides, amino resins, phenylene oxide resins, terephthalic acid resins, epoxy resins, phenolic resins, polystyrene and acrylonitrile copolymers, polyvinylchloride, vinylchloride and vinyl acetate copolymers, acrylate copolymers, alkyd resins, cellulosic film formers, poly(amideimide), styrene-butadiene copolymers, vinylidenechloride/vinylchloride copolymers, vinylacetate/vinylidene chloride copolymers, styrene-alkyd resins, and the like. Another film-forming polymer binder is PCZ-400 (poly(4,4'-dihydroxy-diphenyl-1-1-cyclohexane) which has a viscosity-molecular weight of 40,000 and is available from Mitsubishi Gas Chemical Corporation (Tokyo, Japan).

The charge generating material can be present in the resinous binder composition in various amounts. Generally, at least about 5 percent by volume, or no more than about 90 percent by volume of the charge generating material is dispersed in at least about 95 percent by volume, or no more than about 10 percent by volume of the resinous binder, and more specifically at least about 20 percent, or no more than about 60 percent by volume of the charge generating material is dispersed in at least about 80 percent by volume, or no more than about 40 percent by volume of the resinous binder composition.

In specific embodiments, the charge generation layer 18 may have a thickness of at least about 0.1 µm, or no more than about 2 µm, or of at least about 0.2 µm, or no more than about 1 µm. These embodiments may be comprised of chlorogallium phthalocyanine or hydroxygallium phthalocyanine or mixtures thereof. The charge generation layer 18 containing the charge generating material and the resinous binder material generally ranges in thickness of at least about 0.1 µm, or no more than about 5 µm, for example, from about 0.2 µm to about 3 µm when dry. The charge generation layer thickness is generally related to binder content. Higher binder content compositions generally employ thicker layers for charge generation.

The Charge Transport Layer

In a drum photoreceptor, the charge transport layer comprises a single layer of the same composition. As such, the charge transport layer will be discussed specifically in terms of a single layer 20, but the details will be also applicable to an embodiment having dual charge transport layers. The charge transport layer 20 is thereafter applied over the charge generation layer 18 and may include any suitable transparent organic polymer or non-polymeric material capable of supporting the injection of photogenerated holes or electrons from the charge generation layer 18 and capable of allowing the transport of these holes/electrons through the charge transport layer to selectively discharge the surface charge on the imaging member surface. In one embodiment, the charge transport layer 20 not only serves to transport holes, but also protects the charge generation layer 18 from abrasion or chemical attack and may therefore extend the service life of the imaging member. The charge transport layer 20 can be a substantially non-photoconductive material, but one which supports the injection of photogenerated holes from the charge generation layer 18.

The layer 20 is normally transparent in a wavelength region in which the electrophotographic imaging member is to be used when exposure is affected there to ensure that most of the incident radiation is utilized by the underlying charge generation layer 18. The charge transport layer should exhibit excellent optical transparency with negligible light absorption and no charge generation when exposed to a wavelength of light useful in xerography, e.g., 400 to 900 nanometers. In the case when the photoreceptor is prepared with the use of a transparent substrate 10 and also a transparent or partially transparent conductive layer 12, image wise exposure or erase may be accomplished through the substrate 10 with all light passing through the back side of the substrate. In this case, the materials of the layer 20 need not transmit light in the wavelength region of use if the charge generation layer 18 is sandwiched between the substrate and the charge transport layer 20. The charge transport layer 20 in conjunction with the charge generation layer 18 is an insulator to the extent that an electrostatic charge placed on the charge transport layer is not conducted in the absence of illumination. The charge transport layer 20 should trap minimal charges as the charge passes through it during the discharging process.

The charge transport layer 20 may include any suitable charge transport component or activating compound useful as an additive dissolved or molecularly dispersed in an electrically inactive polymeric material, such as a polycarbonate binder, to form a solid solution and thereby making this material electrically active. "Dissolved" refers, for example, to forming a solution in which the small molecule is dissolved in the polymer to form a homogeneous phase; and molecularly dispersed in embodiments refers, for example, to charge transporting molecules dispersed in the polymer, the small molecules being dispersed in the polymer on a molecular scale. The charge transport component may be added to a film forming polymeric material which is otherwise incapable of supporting the injection of photogenerated holes from the charge generation material and incapable of allowing the transport of these holes through. This addition converts the electrically inactive polymeric material to a material capable of supporting the injection of photogenerated holes from the charge generation layer 18 and capable of allowing the transport of these holes through the charge transport layer 20 in order to discharge the surface charge on the charge transport layer. The high mobility charge transport component may comprise small molecules of an organic compound which cooperate to transport charge between molecules and ultimately to the surface of the charge transport layer. For example, but not limited to, N,N'-diphenyl-N,N-bis(3-methyl phenyl)-1,1'-biphenyl-4,4'-diamine (TPD), other arylamines like triphenyl amine, N,N,N',N'-tetra-p-tolyl-1,1'-biphenyl-4,4'-diamine (TM-TPD), and the like.

A number of charge transport compounds can be included in the charge transport layer, which layer generally is of a thickness of from about 5 to about 75 micrometers, and more specifically, of a thickness of from about 15 to about 40 micrometers. Examples of charge transport components are aryl amines of the following formulas/structures: wherein X is a suitable hydrocarbon like alkyl, alkoxy, aryl, and derivatives thereof; a halogen, or mixtures thereof, and especially those substituents selected from the group consisting of Cl and CH₃; and molecules of the following formulas and wherein X, Y and Z are independently alkyl, alkoxy, aryl, a halogen, or mixtures thereof, and wherein at least one of Y and Z are present.

Alkyl and alkoxy contain, for example, from 1 to about 25 carbon atoms, and more specifically, from 1 to about 12 carbon atoms, such as methyl, ethyl, propyl, butyl, pentyl, and the corresponding alkoxides. Aryl can contain from 6 to about 36 carbon atoms, such as phenyl, and the like. Halogen includes chloride, bromide, iodide, and fluoride. Substituted alkyls, alkoxys, and aryls can also be selected in embodiments.

Examples of specific aryl amines that can be selected for the charge transport layer include N,N'-diphenyl-N,N'-bis(alkylphenyl)-1,1-biphenyl-4,4'-diamine wherein alkyl is selected from the group consisting of methyl, ethyl, propyl, butyl, hexyl, and the like; N,N'-diphenyl-N,N'-bis(halophenyl)-1,1'-biphenyl-4,4'-diamine wherein the halo substituent is a chloro substituent; N,N'-bis(4-butylphenyl)-N,N'-di-p-tolyl-[p-terphenyl]-4,4"-diamine, N,N'-bis(4-butylphenyl)-N,N'-di-m-tolyl-[p-terphenyl]-4,4"-diamine, N,N'-bis(4-butylphenyl)-N,N'-di-o-tolyl-[p-terphenyl]-4,4"-diamine, N,N'-bis(4-butylphenyl)-N,N'-bis-(4-isopropylphenyl)-[p-terphenyl]-4,4"-diamine, N,N'-bis(4-butylphenyl)-N,N'-bis-(2-ethyl-6-methylphenyl)-[p-terphenyl]-4,4"-diamine, N,N'-bis(4-butylphenyl)-N,N'-bis-(2,5-dimethylphenyl)-[p-terphenyl]-4,4'-diamine, N,N'-diphenyl-N,N'-bis(3-chlorophenyl)-[p-terphenyl]-4,4"-diamine, and the like. Other known charge transport layer molecules may be selected in embodiments, reference for example, U.S. Patents 4,921,773 and 4,464,450.

Examples of the binder materials selected for the charge transport layers include components, such as those described in U.S. Patent 3,121,006. Specific examples of polymer binder materials include polycarbonates, polyarylates, acrylate polymers, vinyl polymers, cellulose polymers, polyesters, polysiloxanes, polyamides, polyurethanes, poly(cyclo olefins), and epoxies, and random or alternating copolymers thereof. In embodiments, the charge transport layer, such as a hole transport layer, may have a thickness of at least about 10 µm, or no more than about 40 µm.

Examples of components or materials optionally incorporated into the charge transport layers or at least one charge transport layer to, for example, enable improved lateral charge migration (LCM) resistance include hindered phenolic antioxidants such as tetrakis methylene(3,5-di-tert-butyl-4-hydroxy hydrocinnamate) methane (IRGANOX® 1010, available from Ciba Specialty Chemical), butylated hydroxytoluene (BHT), and other hindered phenolic antioxidants including SUMILIZER™ BHT-R, MDP-S, BBM-S, WX-R, NW, BP-76, BP-101, GA-80, GM and GS (available from Sumitomo Chemical Co., Ltd.), IRGANOX® 1035, 1076, 1098, 1135, 1141, 1222, 1330, 1425WL, 1520L, 245, 259, 3114, 3790, 5057 and 565 (available from Ciba Specialties Chemicals), and ADEKA STAB™ AO-20, AO-30, AO-40, AO-50, AO-60, AO-70, AO-80 and AO-330 (available from Asahi Denka Co., Ltd.);, hindered amine antioxidants such as SANOL™ LS-2626, LS-765, LS-770 and LS-744 (available from SANKYO CO., Ltd.), TINUVIN® 144 and 622LD (available from Ciba Specialties Chemicals), MARK™ LA57, LA67, LA62, LA68 and LA63 (available from Asahi Denka Co., Ltd.), and SUMILIZER® TPS (available from Sumitomo Chemical Co., Ltd.);, thioether antioxidants such as SUMILIZER® TP-D (available from Sumitomo Chemical Co., Ltd);, phosphite antioxidants such as MARK™ 2112, PEP-8, PEP-24G, PEP-36, 329K and HP-10 0 (available from Asahi Denka Co., Ltd.); other molecules such as bis(4-diethylamino-2-methylphenyl) phenylmethane (BDETPM), bis-[2-methyl-4-(N-2-hydroxyethyl-N-ethyl-aminophenyl)]-phenylmethane (DHTPM), and the like. The weight percent of the antioxidant in at least one of the charge transport layer is from about 0 to about 20, from about 1 to about 10, or from about 3 to about 8 weight percent.

The charge transport layer should be an insulator to the extent that the electrostatic charge placed on the hole transport layer is not conducted in the absence of illumination at a rate sufficient to prevent formation and retention of an electrostatic latent image thereon. The charge transport layer is substantially nonabsorbing to visible light or radiation in the region of intended use, but is electrically "active" in that it allows the injection of photogenerated holes from the photoconductive layer, that is the charge generation layer, and allows these holes to be transported through itself to selectively discharge a surface charge on the surface of the active layer.

In addition, in the present embodiments using a belt configuration, the charge transport layer may consist of a single pass charge transport layer or a dual pass charge transport layer (or dual layer charge transport layer) with the same or different transport molecule ratios. In these embodiments, the dual layer charge transport layer has a total thickness of from about 10 µm to about 40 µm. In other embodiments, each layer of the dual layer charge transport layer may have an individual thickness of from 2 µm to about 20 µm. Moreover, the charge transport layer may be configured such that it is used as a top layer of the photoreceptor to inhibit crystallization at the interface of the charge transport layer and the overcoat layer. In another embodiment, the charge transport layer may be configured such that it is used as a first pass charge transport layer to inhibit microcrystallization occurring at the interface between the first pass and second pass layers.

In specific embodiments, the charge transport layer is imprinted on its surface with a nano- to micron-scale pattern. The imprinted surface offers numerous unexpected benefits such as, for example, lower friction with the cleaning blade, improved print quality and smoother interaction to minimize blade damage, and consequently longer service life.

The present embodiments thus provide an imaging member comprising a substrate, a charge generation layer disposed on the substrate, and a charge transport layer disposed on the charge generation layer, wherein the charge transport layer comprises a surface pattern imprinted on a nano- or micron-scale. The surface pattern may include specific shapes and dimensions. For example, the surface pattern may comprise circles, rods, squares, triangles, polygons, mixtures thereof, and the like. In one embodiment, the surface pattern may include one or more indentations. In embodiments, the surface pattern may include an array of indentations having a depth of from about 5 nanometers to about 5 microns, or from 10 nanometers to about 5 microns, or from about 50 nanometers to about 5 microns, or from about 100 nanometers to about 2 microns. In embodiments, the surface pattern comprises an array of indentations having a diameter of from about 5 nanometers to about 100 microns, or from about 10 nanometers to about 100 microns. In other embodiments, the array of indentations have a center-to-center distance of from about 5 nanometers to about 500 microns, or from about 10 nanometers to about 100 microns.

The surface pattern may include indentations being of equidistance from one another in an evenly distributed pattern across the surface of the charge transport layer of the photoreceptor and forming a uniform roughened pattern on the surface of the photoreceptor. The indentations may be in the shape of circles, rods, squares, triangles, polygons, mixtures thereof, and the like.

The present embodiments are made by a method that comprises forming the charge transport layer having the imprinted surface pattern through use of a fabricated mold. For example, the present embodiments provide for a method for forming a photoreceptor charge transport layer, comprising providing a mold for imprinting, wherein the mold is fabricated by printing a pattern on a nano- or micron-scale on a substrate to produce a master pattern, and curing a flexible material onto the master pattern to form the mold, providing a charge transport layer coating for being imprinted, laying the mold over the charge transport layer coating for contacting until the mold and the charge transport layer coating is cross-linked, and removing the mold from the charge transport layer coating such that a charge transport layer comprising a surface pattern imprinted on a nano- or micron-scale is formed.

Any suitable and conventional technique may be utilized to form and thereafter apply the charge transport layer mixture to the supporting substrate layer. The charge transport layer may be formed in a single coating step or in multiple coating steps. Dip coating, ring coating, spray, gravure or any other drum coating methods may be used.

Drying of the deposited coating may be effected by any suitable conventional technique such as oven drying, infra red radiation drying, air drying and the like. The thickness of the charge transport layer after drying is from about 10 µm to about 40 µm or from about 12 µm to about 36 µm for optimum photoelectrical and mechanical results. In another embodiment the thickness is from about 14 µm to about 36 µm.

The Adhesive Layer

An optional separate adhesive interface layer may be provided in certain configurations, such as for example, in flexible web configurations. In the embodiment illustrated in FIG. 1, the interface layer would be situated between the blocking layer 14 and the charge generation layer 18. The interface layer may include a copolyester resin. Exemplary polyester resins which may be utilized for the interface layer include polyarylatepolyvinylbutyrals, such as ARDEL POLYARYLATE (U-1 00) commercially available from Toyota Hsutsu Inc., VITEL PE-1 00, VITEL PE-200, VITEL PE-200D, and VITEL PE-222, all from Bostik, 49,000 polyester from Rohm Hass, polyvinyl butyral, and the like. The adhesive interface layer may be applied directly to the hole blocking layer 14. Thus, the adhesive interface layer in embodiments is in direct contiguous contact with both the underlying hole blocking layer 14 and the overlying charge generator layer 18 to enhance adhesion bonding to provide linkage. In yet other embodiments, the adhesive interface layer is entirely omitted.

Any suitable solvent or solvent mixtures may be employed to form a coating solution of the polyester for the adhesive interface layer. Solvents may include tetrahydrofuran, toluene, monochlorbenzene, methylene chloride, cyclohexanone, and the like, and mixtures thereof. Any other suitable and conventional technique may be used to mix and thereafter apply the adhesive layer coating mixture to the hole blocking layer. Application techniques may include spraying, dip coating, roll coating, wire wound rod coating, and the like. Drying of the deposited wet coating may be effected by any suitable conventional process, such as oven drying, infra red radiation drying, air drying, and the like.

The adhesive interface layer may have a thickness of at least about 0.01 micrometers, or no more than about 900 micrometers after drying. In embodiments, the dried thickness is from about 0.03 micrometers to about 1 micrometer.

The Ground Strip

The ground strip may comprise a film forming polymer binder and electrically conductive particles. Any suitable electrically conductive particles may be used in the electrically conductive ground strip layer 19. The ground strip 19 may comprise materials which include those enumerated in U.S. Pat. No. 4,664,995. Electrically conductive particles include carbon black, graphite, copper, silver, gold, nickel, tantalum, chromium, zirconium, vanadium, niobium, indium tin oxide and the like. The electrically conductive particles may have any suitable shape. Shapes may include irregular, granular, spherical, elliptical, cubic, flake, filament, and the like. The electrically conductive particles should have a particle size less than the thickness of the electrically conductive ground strip layer to avoid an electrically conductive ground strip layer having an excessively irregular outer surface. An average particle size of less than about 10 micrometers generally avoids excessive protrusion of the electrically conductive particles at the outer surface of the dried ground strip layer and ensures relatively uniform dispersion of the particles throughout the matrix of the dried ground strip layer. The concentration of the conductive particles to be used in the ground strip depends on factors such as the conductivity of the specific conductive particles utilized.

The ground strip layer may have a thickness of at least about 7 micrometers, or no more than about 42 micrometers, or of at least about 14 micrometers, or no more than about 27 micrometers.

The Anti-Curl Back Coating Layer

The anti-curl back coating 1 may comprise organic polymers or inorganic polymers that are electrically insulating or slightly semi-conductive. The anti-curl back coating provides flatness and/or abrasion resistance.

Anti-curl back coating 1 may be formed at the back side of the substrate 2, opposite to the imaging layers. The anti-curl back coating may comprise a film forming resin binder and an adhesion promoter additive. The resin binder may be the same resins as the resin binders of the charge transport layer discussed above. Examples of film forming resins include polyacrylate, polystyrene, bisphenol polycarbonate, poly(4,4'-isopropylidene diphenyl carbonate), 4,4'-cyclohexylidene diphenyl polycarbonate, and the like. Adhesion promoters used as additives include 49,000 (du Pont), Vitel PE-1 00, Vitel PE-200, Vitel PE-307 (Goodyear), and the like. Usually from about 1 to about 15 weight percent adhesion promoter is selected for film forming resin addition. The thickness of the anti-curl back coating is at least about 3 micrometers, or no more than about 35 micrometers, or about 14 micrometers.

Various exemplary embodiments encompassed herein include a method of imaging which includes generating an electrostatic latent image on an imaging member, developing a latent image, and transferring the developed electrostatic image to a suitable substrate.

The presently disclosed embodiments are, therefore, to be considered in all respects as illustrative and not restrictive, the scope of embodiments being indicated by the appended claims rather than the foregoing description.

All changes that come within the meaning of and range of equivalency of the claims are intended to be embraced therein.

### EXAMPLES

The examples set forth herein below and is illustrative of different compositions and conditions that can be used in practicing the present embodiments. All proportions are by weight unless otherwise indicated.

**Example 1**

**Fabrication of Mold:**

A photo-mask was fabricated by using a dot inkjet-printer on a transparent substrate to make a master pattern on silicon wafer by photolithography. The printed dot pattern comprised an array of indentations in which the diameter of each indentation was 40 microns and a center-to-center distance between the indentations was 100 microns. First SU-8 resin (available from MicroChem, Newton, MA) was spin-coated on silicon wafer. The SU-8 film was pre-exposure heated at 65 degrees for 30 minutes. The dot printed transparent photo-mask was contacted unto the SU-8 film and exposed for 3 minutes to 100 mW UV light (325 nm). The SU-8 film was then post-exposure heated at 65 degrees for 30 minutes. The SU-8 film was wet-etched by SU-8 developing solvent and followed by washing with iso-propanol to achieve the master pattern. The master pattern was replicated by curing flexible polydimethylsiloxane (PDMS) materials onto the master pattern. The formed mold comprised an array of protrusions, corresponding to the indentations of the master pattern. Each protrusion of the flexible mold had a height of 10 microns. The replicated flexible PDMS mold was used for imprinting directly on top of an overcoat layer. The resulting indentation on top of the overcoat layer had a depth of 1 micron. A depth of 1 micron is reasonable to not smear ink during real printing process. As stated above, however, the design of the master pattern or mold may comprise a variety of shapes, for example, circles, rods, squares, oval, triangles, polygons, mixtures thereof and the like, as well as variable dimensions.

**Fabrication of Cylinder/Drum-type Photoreceptor with Patterned Overcoat Layer:**

An electrophotographic photoreceptor was fabricated in the following manner. A coating solution for an undercoat layer comprising 100 parts of a ziconium compound (trade name: Orgatics ZC540), 10 parts of a silane compound (trade name: A110, manufactured by Nippon Unicar Co., Ltd), 400 parts of isopropanol solution and 200 parts of butanol was prepared. The coating solution was applied onto a cylindrical aluminum (Al) substrate subjected to honing treatment by dip coating, and dried by heating at 150 °C for 10 minutes to form an undercoat layer having a film thickness of 0.1 micrometer.

A 0.5 micron thick charge generating layer was subsequently dip coated on top of the undercoat layer from a dispersion of Type V hydroxygallium phthalocyanine (12 parts), alkylhydroxy gallium phthalocyanine (3 parts), and a vinyl chloride/vinyl acetate copolymer, VMCH (Mn = 27,000, about 86 weight percent of vinyl chloride, about 13 weight percent of vinyl acetate and about 1 weight percent of maleic acid) available from Dow Chemical (10 parts), in 475 parts of n-butylacetate.

Subsequently, a 25 µm thick charge transport layer (CTL) was dip coated on top of the charge generating layer from a solution of N,N'-diphenyl-N,N'-bis(3-methylphenyl)-1,1'-biphenyl-4,4'-diamine (82.3 parts), 2.1 parts of 2,6-di-tert-butyl-4-methylphenol (BHT) from Aldrich and a polycarbonate, PCZ-400 [poly(4,4'-dihydroxydiphenyl-1-1-cyclohexane), M_{w} = 40,000] available from Mitsubishi Gas Chemical Company, Ltd. (123.5 parts) in a mixture of 546 parts of tetrahydrofuran (THF) and 234 parts of monochlorobenzene. The CTL was dried at 115°C for 60 minutes.

An overcoat formulation was prepared from a mixture of an acrylic polyol (1.5 parts, JONCRYL-587, available from Johnson Polymers LLC, Sturtevant, Wisconsin, USA), a melamine resin (2.1 parts, CYMEL-303 available from Cytec Industries, Inc. West Paterson, New Jersey, USA), a charge transport component of N,N,N',N'-tetrakis-[(4-hydroxymethyl)phenyl]-biphenyl-4,4'-diamine (THM-TBD)(1.16 parts)/ N,N'-diphenyl-N,N'-di(3-hydroxyphenyl)-terphenyl-diamine (DHTER)(1.93 pats), and an acid catalyst (0.05 part, Nacure 5225 available from King Chemical Industries), in a solvent of 1-methoxy-2-propanol (20.9 parts). The solution was applied onto the photoreceptor surface and more specifically onto the charge transport layer, using cup coating technique, followed by micro/nano imprinting with the flexible mold. The possible imprinting time window before the overcoat material dried was about 3 minutes. Finally thermal curing was done at 140 °C for 40 minutes to form an imprinted overcoat layer having an average film thickness of about 6 µm. For demonstration and comparison experiments, each drum was imprinted twice for a certain width, *e.g*, 4 cm width and 5 cm width, with a non-imprinted reference width in between the two imprinted widths. From an engineering point of view, the micro/nano imprinting can be implemented through efficient roll-to-roll process.

**Comparative Example:**

An electrophotographic photoreceptor having an overcoat comprising no patterns was fabricated in a similar manner as described in Example 1 except that no pattern was imprinted in the preparation of overcoat layer.

**Evaluation of Electrophotographic Photoreceptor Performance:**

The electrical performance characteristics of the above prepared electrophotographic photoreceptors such as electrophotographic sensitivity and short term cycling stability were tested in a scanner. The scanner is known in the industry and equipped with means to rotate the drum while it is electrically charged and discharged. The charge on the photoconductor sample is monitored through use of electrostatic probes placed at precise positions around the circumference of the device. The photoreceptor devices are charged to a negative potential of 500 Volts. As the devices rotate, the initial charging potentials are measured by voltage probe 1. The photoconductor samples are then exposed to monochromatic radiation of known intensity, and the surface potential measured by voltage probes 2 and 3. Finally, the samples are exposed to an erase lamp of appropriate intensity and wavelength and any residual potential is measure by voltage probe 4. The process is repeated under the control of the scanner's computer, and the data is stored in the computer. The PIDC (photo induced discharge curve) is obtained by plotting the potentials at voltage probes 2 and 3 as a function of the light energy. All the photoreceptors as prepared in Examples 1 and 2, showed similar PIDC characteristics as the control or Comparative Example device. The test results, in Table 1, demonstrate that the electrical performance of the imprinted samples is nearly same with that of the non-imprinted reference sample.

**Table 1.**

| | Reference 1 | Sample 1 | Sample 2 | Reference 2 | Sample 3 | Sample 4 |
|---|---|---|---|---|---|---|
| V(3) | 314 | 302 | 308 | 307 | 314 | 309 |
| V(10) | 112 | 107 | 110 | 108 | 112 | 109 |

**Torque Measurements:**

The measurements were made on a control drum without an overcoat, a drum with a non-patterned overcoat, and two imprinted drums. Multiple measurements were made and averaged. Results, shown in FIG. 4, clearly indicate that the micro/nano imprinted drums showed lower torque than the non-patterned overcoat drum. Wider (5 cm width) region imprinted drum shows 40% reduction in torque over the non-patterned overcoat drum.

Future optimization on the design of pattern and size of the particular surface pattern on the master pattern is possible for maximum torque reduction. Initial print tests showed good solid-area, halftone and line reproduction, similar to the control. No major print defect occurred to the presence of the periodic imprinted pattern.

In summary, this invention describes a micro/nano imprinting of overcoat surface that enables reduced torque through "periodically patterned" surface morphology of photoreceptor surface. The micro/nano imprinting method is simple and reproducible with reusable mold and important to control homogeneously on top of photoreceptor surface and to guide morphology during cycled wear of photoreceptor surface.

**Example 2**

**Fabrication of Belt-type Photoreceptor with Patterned CTL Layer:**

An imaging or photoconducting member was prepared in accordance with the following procedure. A metallized MYLAR substrate was provided and a HOGaPc/poly(bisphenol-Z carbonate) photogenerating layer was machine coated over the substrate. The photogenerating layer was coated with a charge transport layer prepared by introducing into an amber glass bottle about 50 weight percent of N,N'-(3-methylphenyl)-N,N'-diphenyl-1,1'-biphenyl-4,4'-diamine, 5 weights of an anti-oxidant, and 45 weight percent of MAKROLON 5705, a known polycarbonate resin having a molecular weight average of from about 50,000 to about 100,000, commercially available from Farbenfabriken Bayer A.G. The resulting mixture was then dissolved in methylene chloride to form a solution containing 15 percent by weight solids. This solution was applied on the photogenerating layer to form a layer coating, followed by being covered and imprinted with PDMS mold, which was replicated from the master pattern by photolithography. By pressing with moderate pressure, the surface pattern was imprinted on the CTL. After final curing of the CTL (120°C for 1 minute), the surface pattern of an array of indentations remained permanently on the CTL. The hole depth was 1 micron and the diameter was 40 microns. During this coating and imprinting processes, the humidity was equal to or less than about 15 percent.

**Comparative Example:**

An electrophotographic photoreceptor having an CTL comprising no patterns was fabricated in a similar manner as described in Example 2 except that no pattern was imprinted in the preparation of CTL layer.

**Evaluation of Electrophotographic Photoreceptor Performance:**

Two sets of samples were prepared - one control sample (no pattern) and one patterned sample. The samples were cut into three equally sized strips and mounted on an 84 mm (uncoated) drum in a 6X configuration for concurrent evaluation in a drum scanner. The control was represented by the a, b and c strips, and the patterned sample was represented by the d, e and f strips are the patterned samples.

PIDCs were taken at time-zero under standard conditions to check for reproducibility and uniformity. Long term (30K) electrical cycling was then performed - during this cycling only the b and e strips are subjected to positive charge stress. The bracketing strips (a, c and d, f) provide a baseline reference. All samples are subjected to the same negative charge and exposure during this cycling. Finally, PIDCs were taken post-cycling and the positive charge stressed strips are compared with the non-positive charge strips. The results are shown in Tables 2 (PIDC parameters: time zero measurement and output voltage (Vₒ)) and 3 below (PIDC parameters: post-30K cycling stress, positive charge on b and e only, Vₒ held constant with feedback).

**Table 2.**

| Photoreceptor Sample | a | b | c | d | e | f |
|---|---|---|---|---|---|---|
| Vₒ^{*} (V) | 487 | 487 | 487 | 490 | 484 | 485 |
| Vᵣ^{*} (V) | 14 | 12 | 9 | 12 | 17 | 10 |
| V_{c}^{*} (V) | 121 | 120 | 121 | 130 | 121 | 121 |
| S^{*} (cm²/erg) | 393 | 396 | 427 | 444 | 402 | 421 |
| E_{1/2}^{*} (erg/cm²) | 0.70 | 0.70 | 0.64 | 0.64 | 0.69 | 0.65 |
| E_{7/8}^{*} (erg/cm²) | 1.79 | 1.75 | 1.59 | 1.65 | 1.81 | 1.63 |
| ESV 5 (avg) (V) | 12 | 11 | 9 | 10 | 13 | 9 |
| ESV 1 (avg) (V) | 545 | 543 | 537 | 537 | 546 | 533 |
| ESV 2 (avg) (V) | 520 | 519 | 516 | 517 | 520 | 513 |
| DD (ESV1-2) (V) | 25 | 23 | 22 | 20 | 26 | 21 |

| | | | | | | |
|---|---|---|---|---|---|---|
| * fitted parameters ESV3 | | | | | | |

**Table 3.**

| Photoreceptor Sample | a | b | c | d | e | f |
|---|---|---|---|---|---|---|
| Vₒ^{*} (V) | 497 | 499 | 498 | 498 | 499 | 499 |
| Vᵣ^{*} (V) | 44 | 27 | 36 | 37 | 35 | 31 |
| V_{c}^{*} (V) | 140 | 125 | 141 | 150 | 122 | 146 |
| S^{*} (cm²/erg) | 347 | 369 | 379 | 383 | 371 | 371 |
| E_{1/2}^{*} (erg/cm²) | 0.87 | 0.77 | 0.79 | 0.80 | 0.77 | 0.81 |
| E_{7/8}^{*} (erg/cm²) | 4.14 | 2.27 | 3.01 | 3.33 3 | 2.56 | 2.89 |
| ESV 5 (avg) (V) | 31 | 22 | 24 | 22 | 28 | 19 |
| ESV 1 (avg) (V) | 551 | 559 | 542 | 540 | 566 | 545 |
| ESV 2 (avg) (V) | 527 | 533 | 522 | 521 | 537 7 | 524 |
| DD (ESV1-2) (V) | 24 | 27 | 19 | 19 | 29 | 21 |

| | | | | | | |
|---|---|---|---|---|---|---|
| * fitted parameters ESV3 Vₒ is the dark voltage after scorotron charging; Vr is the residual potential after light erase; Vc is the potential at the half way point of slope S; S is the initial slope of the PIDC curve and is a measurement of sensitivity; E_{1/2} and E_{7/8} are exposure amounts; and ESV stands for electrostatic voltmeter. | | | | | | |

Photodischarge characteristics are represented by E_{1/2} and E_{7/8} values. E_{1/2} is the exposure energy required to achieve a photodischarge from the dark development potential (V_{ddp}) to 1/2 of V_{ddp} and E_{7/8} the energy for a discharge from V_{ddp} to 1 /8 of V_{ddp}. The light energy used to photodischarge the imaging member during the exposure step was measured with a light meter. The higher the photosensitivity, the smaller are E_{1/2} and E_{7/8} values.

FIG. 5 shows the significantly reduced PEG behavior of the patterned sample. The PEG signal shows that there is significant improvement in the tail region of the PIDC (above 2.0 erg/cm²). In embodiments, the improved imaging member exhibits from about 10% to about 90% reduction in paper edge ghost as compared to an imaging member comprising a charge transport layer without the surface pattern. For example, the patterned sample shows half as much differential cycle-up as the control sample. It must be noted that the nano- or micron-scale patterning improvements against PEG can be applied to belt architectures as well as to drums.

In summary, this invention describes a micro/nano imprinting of charge transport layer surface that enables reduced PEG through "periodically patterned" surface morphology of photoreceptor surface. As stated above, the micro/nano imprinting method is simple and reproducible with reusable mold and important to control homogeneously on top of photoreceptor surface and to guide morphology during cycled wear of photoreceptor surface.

## Claims

1. An imaging member comprising:
a substrate;
a photosensitive layer disposed on the substrate; and
an outer layer disposed on the photosensitive layer, wherein the outer layer of the imaging member has a patterned surface comprising an array of periodically ordered indentations or protrusions on the surface of the outer layer.

2. The imaging member of claim 1, wherein the indentations or protrusions have a regular shape selected from the group consisting of circles, rods, ovals, squares, triangles, polygons, and mixtures thereof, or
wherein each of the indentations or protrusions has a perimeter from about 5 nanometers to about 200 microns, or
wherein the indentations have a depth of from about 5 nanometers to about 5 microns, and the protrusions have height of from about 5 nanometers to about 5 microns.

3. The imaging member of claim 1, wherein the array of indentations or protrusions are regularly positioned over the surface of the outer layer, or
wherein the indentations or protrusions have a two-dimensional periodicity from hexagonal arrays, tetragonal arrays, quasi-crystal arrays, and linear arrays, and mixtures thereof, or
wherein the array of indentations or protrusions have a center-to-center distance of from about 5 nanometers to about 500 microns.

4. The imaging member of claim 1, wherein the photosensitive layer further comprises a charge generation layer disposed on the substrate and a charge transport layer disposed on the charge generation layer, wherein the charge generation layer comprises a photosensitive pigment and the charge transport layer is the outer layer of the imaging member, optionally
wherein the photosensitive pigment is selected from the group consisting of metal free phthalocyanine, titanyl phthalocyanine, chlorogallium phthalocyanine, hydroxygallium phthalocyanine, and a mixture of alkylhydroxy gallium phthalocyanine and hydroxygallium phthalocyanine, and a perylene, and further wherein the charge transport layer comprises a tertiary arylamine selected from the group consisting of N,N'-diphenyl-N,N'-bis(3-methylphenyl)-(1,1'-biphenyl)-4,4'-diamine, N,N'-diphenyl-N,N'-bis(4-methylphenyl)-(1,1'-biphenyl)-4,4'-diamine, N,N,N',N'-tetrakis(4-methylphenyl)-1,1'-biphenyl)-4,4'-diamine, N,N'-bis(4-butylphenyl)-N,N'-di-p-tolyl-[p-terphenyl]-4,4'-diamine, and N,N'-bis(4-butylphenyl)-N,N'-di-m-tolyl-[p-terphenyl]-4,4'-diamine, and mixtures thereof.

5. The imaging member of claim 1, wherein the photosensitive layer further comprises a charge generation layer disposed on the substrate, a charge transport layer disposed on the charge generation layer, and an overcoat layer disposed on the charge transport layer, wherein the overcoat layer is the outer layer of the imaging member.

6. The imaging member of claim 5, wherein the charge generation layer comprises a photosensitive pigment selected from the group consisting of metal free phthalocyanine, titanyl phthalocyanine, chlorogailium phthalocyanine, hydroxygallium phthalocyanine, and a mixture of alkylhydroxy gallium phthalocyanine and hydroxygallium phthalocyanine, and a perylene, and the charge transport layer comprises a tertiary arylamine selected from the group consisting of N,N'-diphenyl-N,N'-bis(3-methylphenyl)-(1,1'-biphenyl)-4,4'-diamine, N,N'-diphenyl-N,N'-bis(4-methylphenyl)-(1,1'-biphenyl)-4,4'-diamine, N,N,N',N'-tetrakis(4-methylphenyl)- 1,1'-biphenyl)-4,4'-diamine, N,N'-bis(4-butylphenyl)-N,N'-di-p-tolyl-[p-terphenyl]-4,4'-diamine, and N,N'-bis(4-butylphenyl)-N,N'-di-m-tolyl-[p-terphenyl]-4,4'-diamine, and mixtures thereof

7. The imaging member of claim 5, wherein the overcoat layer comprises a cross-linked composition further comprising a charge transport component.

8. The imaging member of claim 7, wherein the cross-linked composition is achieved by curing and polymerization of a charge transport component comprised of a tertiary arylamine having at least a curable functional group selected from the group consisting of a hydroxyl, a hydroxymethyl, an alkoxymethyl, a hydroxyalkyl having from 1 to about 15 carbons, an acrylate, and the mixture thereof.

9. The imaging member of claim 8, wherein an additional curing agent is added for forming the cross-linked composition.

10. The imaging member of claim 9, wherein the curing agent is selected from the group consisting of a melamine-formaldehyde resin, a phenol resin, an isocyalate or a masking isocyalate compound, an acrylate resin, a polyol resin, or the mixture thereof.

11. The imaging member of claim 1, being in a belt, a drum, or a plate configuration.

12. An imaging member according to claim 4 comprising:
a substrate;
a charge generation layer disposed on the substrate; and
a charge transport layer disposed on the charge generation layer, wherein the charge transport layer has a patterned surface comprising an array of periodically ordered indentations or protrusions on the surface of the outer layer and further wherein the charge transport layer comprises a tertiary arylamine and an optional polymer binder present in a ratio amount of from about 10/90 to about 90/10.

13. An image forming apparatus comprising:
an imaging member according to claim 1;
a charging unit that applies electrostatic charge on the imaging member;
a developing unit that develops toner image onto the imaging member;
a transfer unit that transfers the toner image from the imaging member to a media; and
a cleaning unit that cleans the imaging member.

14. The image forming apparatus of claim 13, wherein the indentations or protrusions have a depth or height of from about 0.1 micrometer to about 5 microns, wherein the array of indentations or protrusions each have a perimeter of from about 0.1 micrometer to about 200 microns, and wherein the array of indentations or protrusions have a center-to-center distance of from about 0.5 micrometer to about 200 microns.

15. The image forming apparatus of claim 13, wherein the cleaning unit comprises a blade-type cleaner comprising an elastic polymer.
